

# UNITED STATES PATENT OFFICE.

HEINRICH BERNHARD AND OSKAR JAECK, OF BASEL, SWITZERLAND, ASSIGNORS TO  
SOCIETY OF CHEMICAL INDUSTRY IN BASLE, OF BASEL, SWITZERLAND.

## PROCESS FOR DEGUMMING RAW SILK IN PRESENCE OF VAT-DYED SILK.

1,409,653.

Specification of Letters Patent. Patented Mar. 14, 1922.

No Drawing.

Application filed September 13, 1921. Serial No. 500,375.

To all whom it may concern:

Be it known that we, HEINRICH BERNHARD and OSKAR JAECK, both citizens of the Swiss Republic, and residents of Basel, Switzerland, have invented a new and useful Process for Degumming Raw Silk in Presence of Vat-Dyed Silk, of which the following is a full, clear, and exact specification.

10 When, according to the usual methods, one essays to degum or ungum raw silk with a hot soap solution in presence of silk dyed with vat-dyestuffs, one observes often that the dyestuff of the vat-dyed silk is 15 partly reduced and runs or is disgorged more or less in the silk subjected to the ungumming.

If, searching to obviate this drawback, an oxidizing agent, as hydrogen peroxide or 20 an alkali metal perborate, be added to the ungumming bath, no appreciable improvement is observed. In the course of our investigations, we have found, that this inconvenience can be avoided, if a small 25 quantity of an alkali metal persulfate is added to the soapy degumming bath. This addition prevents the reduction of such vat dyestuffs which are sensitive to the action of the degumming bath and therefore such 30 dyestuffs can thus be employed for fancy coloured woven fabrics.

### Example.

1 part of silk dyed with ciba violet B and 10 parts of raw silk are boiled together, for 2 hours, in a degumming bath containing 35 15 gr. of soap of Marseille and 2 gr. of potassium persulfate per liter. No reduction of the dyestuff is observed and the silk, which has been ungummed, remains 40 white. An analogous result is obtained with other vat-dyestuffs, as for instance ciba-brown B, ciba-grey C, helindon-pink AN, helindon-scarlet R.

### What we claim is:

The herein described process for degumming raw silk in presence of vat-dyed silk wherein an alkali-metal persulfate is added to the ungumming bath, thus preventing the vat-dyestuff from being reduced and running onto the undyed silk during the 50 process of ungumming.

In witness whereof we have hereunto signed our names this 27th day of August, 1921, in the presence of two subscribing witnesses.

HEINRICH BERNHARD.  
OSKAR JAECK.

### Witnesses:

FRISCHER KURZ,  
AMAND RITTER.